

Feb. 22, 1944.

B. H. MACKEY

2,342,204

METHOD OF MANUFACTURING SMOKELESS POWDER

Filed March 27, 1940



Bill Harry Mackey

INVENTOR

BY Thos. A. Wilson

ATTORNEY

## UNITED STATES PATENT OFFICE

2,342,204

## METHOD OF MANUFACTURING SMOKELESS POWDER

Bill Harry Mackey, Wilmington, Del., assignor to  
E. I. du Pont de Nemours & Company, Wil-  
mington, Del., a corporation of Delaware

Application March 27, 1940, Serial No. 326,162

4 Claims. (Cl. 18—55)

This invention pertains to a process of making smokeless powder and more particularly to a smokeless powder in the form of grains having definite dimensions, said powder possessing enhanced mechanical strength.

The chief advantage of producing powder grains of predetermined size and shape, and having perforations of exact size, lies in the fact that such grains permit some control over the burning of the powder and consequently over its ballistic performance. Thus, the perforations of any particular grain are designed to afford an increase in the burning surface as the grain burns, and hence are deemed an important factor in maintaining what is considered the optimum burning surface during the various stages of the powder's combustion.

Heretofore, smokeless powders of this type have been produced by forcing a suitable colloid composition through one or more dies in a press, the colloid issuing from the dies in the form of perforated strands or strings. This process has been characterized by the flow of the colloid in a single direction only. Thus, although many dies involving various modifications with respect to their assembly have been known, all of them permit a substantially straight flow of the colloid along the pins of the die plate and the walls of the die body. Such a conventional die is indicated in several figures of the drawing referred to in the following. After issuing from the conventional die, the strings of colloid are fed to cutters adjusted to cut segments of the desired length. The "green" powder grains are then treated in a system which permits the recovery of the bulk of the solvent, following which they are dried.

The resulting conventional powder grains invariably have exhibited two outstanding defective characteristics: First, the grain has shrunk much more across the diameter or web than it has in length; second, upon impact the grain shows a cleavage along a line parallel to the longitudinal axis of the grain rather than across its diameter.

Such characteristics are undesirable for the reason that the proper ballistic performance of a powder is dependent upon the grains remaining as integral units during the combustion of the charge, rather than breaking into fragments, since fragmentation of said grains exposes burning surface exceeding that calculated as desirable, with the result that erratic ballistic performances are obtained. Actually, such erratic performances heretofore have been common, at

least in certain firearms, the fragmentation of the grains resulting either from the pressure created by the medium of ignition or by the pressure developed by combustion of part of the smokeless powder charge itself.

Various attempts have been made to overcome this undesirable phenomenon, said attempts being directed to a composition better able to withstand the pressures developed, as well as to charges of such design that fragmentation would be less apt to occur. Thus, in order to obtain a tougher composition, varying amounts of gun-cotton and pyrocellulose have been blended, different solvents have been employed, and numerous additional ingredients have been incorporated in the composition. Likewise, experiments have been made wherein the powder charge was arranged with respect to the ignition charge in order to prevent travel of the charge, as by spacers, for example, so that fragmentation would be eliminated or at least diminished appreciably.

The foregoing modifications have in general effected an improvement but in no case can the conventional powder be fired with the certainty that fragmentation and consequent erratic ballistic results will be avoided.

The object of the present invention is a method of pressing smokeless colloids which yields a grain that shrinks substantially uniformly in all dimensions. Other objects will become apparent as the invention is described hereinafter.

I have found that the foregoing objects are accomplished by forming the smokeless powder grain in such manner that there is a random or improved orientation of the particles of material of which the grain is composed.

This may be accomplished by more than one method. For instance, I have found that the two undesirable characteristics mentioned, namely, the uneven shrinkage and extreme fragility can be overcome through that improved particle orientation achieved if, while forming the grain, I prevent flow of the colloid in one direction only. Thus, if in the formation of the final grain, the colloid be moved in a helical or concentric path, the behavior of the finished grain is altered remarkably. The particles then are not aligned in one direction only, but rather point in numerous directions, lying at various angles in many different planes. This disarray of particles I call "random orientation" and this term is used in this sense throughout the description of the invention. The grains wherein the particles have this property are characterized

by uniform shrinkage and greatly enhanced impact resistance.

I have determined that this random orientation of particles may be achieved also by a process different from that employing the helical or concentric path, namely, by charging the colloid into die molds and applying pressure preferably by means of a piston to form the grain of predetermined dimensions.

My invention may be more readily understood by referring to the accompanying drawing. Similar numerals are employed to designate corresponding parts throughout the various figures of the drawing.

Figure 1 is a cross-sectional view in elevation of a die mold according to the present invention. Figure 2 is a cross-sectional view in elevation of a die according to the present invention. Figure 3 is a plan view of the same.

The following example refers in greater detail to Figure 1 of the drawing. This example also brings out the outstanding properties of the powder of my invention.

#### Example

A smokeless powder colloid was prepared in conventional fashion, the various ingredients being mixed with the requisite amount of ether and alcohol. After mixing, the colloid was macerated, pressed into a block, and the block extruded through small orifices, thereby forming the material into strings. A portion of these strings was pressed in a press and extruded through the conventional type of die.

The second portion of the colloid was divided into predetermined quantities and charged into die molds of the type shown in Figure 1, wherein 10 represents a die head having the die pins 11, said die head fitting snugly within the walls 12. Pressure is applied by appropriate means via the piston 13. The particular die molds employed were designed to yield a grain having dimensions identical with those produced above. Both types of grains were dried under identical conditions. In this manner, grains having identical form and shape were produced, the only difference being in the actual formation of the final grain. After all the grains had been dried to the same content of volatile material, they were measured to determine the shrinkage of the various dimensions. The amount of shrinkage as determined from the measurement of numerous grains is given below:

| Grains                            | Shrinkage                                                 |
|-----------------------------------|-----------------------------------------------------------|
|                                   | Percent                                                   |
| A (grains formed in usual manner) | Length 4.10<br>D 21.61<br>d 27.59<br>TW 35.01<br>OW 27.14 |
| B (molded grains)                 | Length 19.4<br>D 19.8<br>d 20.1<br>TW 22.2<br>OW 20.4     |

An examination of the shrinkage results noted above reveals that the A type grains shrunk over 5 times as much in diameter as they did in length, whereas the molded grains (type B) showed that the shrinkage in diameter was approximately equal to that in length.

With respect to resistance to impact, the grains of random orientation showed a strikingly large increase over the ordinary powder grains, even though the design and composition of the grains

are identical. The increased impact resistance is illustrated in the following test:

The dried A and B grains were tested for impact by permitting flat metal weights to fall on the grain which rested on a smooth metal surface. In order to eliminate possible irregularities of the grains, one-half inch sections were taken from each grain, and these sections subjected to the test. The results were as follows:

| Grains | Weight of falling metal | Distance required to crack grains |
|--------|-------------------------|-----------------------------------|
| A      | 0.5<br>1.0              | 26-30<br>13-14                    |
| B      | 0.5<br>1.0              | (1)<br>55-69                      |

<sup>1</sup> No breakage—69" max. ht.

<sup>2</sup> Some grains failed to break when the weight was dropped from the maximum height of 69 inches.

In conducting the impact tests on the A grains, it was noted that the grain cracked almost invariably along the longitudinal plane regardless of the position in which the grain was placed. Whether it was placed with the cross-section uppermost or to one side made no difference. The line of cleavage generally was clean-cut and definite. By contrast, the B grains broke irregularly in a jagged line along no particular plane. The fact that the B grains are much more resistant to impact is shown by the results cited above, said results indicating that this type of grain has about 5 times the impact resistance of the usual grain.

The method or means of procuring random orientation is not limited to the molding of powders by means of a device of the type shown in Figure 1, but may be obtained in numerous manners. For instance, referring in greater detail to Figures 3 and 4, involving the improved die, the colloid is forced through the orifices 15, these being curved so that the material enters the section in which the pins are located at almost right angles to the longitudinal dimension of the pins. The path of the orifices is indicated by the curved passageways 16. Although only one series of orifices is shown (Figure 3), it is clear that more can be added if desired. Undoubtedly, other modifications can be made to cause the material to flow helically or concentrically through the die in order that no substantial alignment of the particles in a single direction results.

Figure 4 is a view, partly in cross-section and partly in perspective, of a string of powder as it is formed when using a die of the type set forth in Figures 2 and 3. It may be seen that the particles of the smokeless powder colloid, due to the direction in which they are forced into the die, take a path which is helical or concentric, so that the string of powder is composed of particles which have not been aligned in one direction only, because, in moving through the die, they are forced therethrough in a tortuous path which may be indicated by the fine lines representing the smokeless powder colloid.

The fact that the prevention of streamline flow of the colloid during formation of the powder grain should cause the properties of the finished grain to be different is very surprising in view of the fact that the usual manufacture of smokeless powder entails working of the colloid to a considerable extent prior to final formation of the grain. Thus, the solvent-laden colloid is

thoroughly mixed, macrated, compressed in a blocking press, and then extruded through small orifices prior to its extrusion in final form. Due to this rather extreme treatment, it commonly was believed that the fibrous structure of the nitrocellulose had been substantially destroyed and that the colloid was essentially homogeneous. Therefore, it was natural in the absence of explanation to consider the non-uniform shrinkage and the definite cleavage along the longitudinal axis of the grain as inherent characteristics of smokeless powder.

I believe that, even though the colloid be homogeneous and composed of particles indiscriminately disarrayed prior to formation of the grain, the passage through the usual die causes substantial alignment of the particles of the colloid in one direction only, this direction being that along the longitudinal axis of the grain. The force necessary to separate the particles is then less than that required to break or sever the particles in a direction cross-wise to the longitudinal axis. Thus, it is logical that the elimination of the solvent by drying would cause greater shrinkage across the diameter than in the length of the grain. Likewise, this would account for the cleavage of the grain along the longitudinal axis of the grain. However, I am unable to prove conclusively the foregoing explanation and since it is a theory, I do not intend to be limited thereby.

At any rate, regardless of theory, it is clear that the methods of my invention as described herein produce a novel form of grain smokeless powder characterized by the fact that the individual grains are uniformly shrunk and are remarkably resistant to impact.

By producing a powder having an impact resistance much greater than powders of similar design and composition, it is possible to decrease and in many cases to eliminate the fragmentation of smokeless powder charges which obtains when they are initiated. Since this change in making the grain does not alter the burning

characteristics, it follows that the erratic ballistic performances due to the fragmentation may be proportionately reduced or eliminated. Likewise, the adoption of grains of this type obviates the necessity of exercising some of the precautions heretofore taken to keep fragmentation to the minimum possible degree, such as spacing of the charge, for example.

It will be evident to those skilled in the smokeless powder art that the foregoing description permits of variations without departing from the spirit or scope of the invention. I intend therefore to be limited only in accordance with the following patent claims:

15 I claim:

1. A method of producing smokeless powder grains having enhanced resistance to fragmentation, which comprises imparting a helical flow to the smokeless powder colloid while extruding said colloid through a die.

2. A method of producing smokeless powder grains having enhanced resistance to fragmentation, which comprises forcing said colloid through a helical path during extrusion of smokeless powder colloid through a die which is adapted to yield a finished grain of the definite dimensions.

3. A method of producing a substantially uniform shrinking smokeless powder grain having increased resistance to impact, which comprises imparting a helical path to the colloid while extruding said colloid through a die of predetermined form.

4. A method of producing a smokeless powder grain of enhanced resistance to fragmentation, which comprises mingling the various ingredients including nitrocellulose with a solvent for said nitrocellulose, forming the solvent-laden mixture into a colloid by exerting work thereon, passing said colloid in a helical path while forcing it through a die adapted to yield the final form of the grain, and drying the grains to a given moisture content.

BILL HARRY MACKEY.

CERTIFICATE OF CORRECTION.

Patent No. 2,342,204.

February 22, 1944.

BILL HARRY MACKEY.

It is hereby certified that error appears in the printed specification of the above numbered patent requiring correction as follows: Page 3, first column, line 1, for "macrated" read --macerated--; and second column, line 23, claim 2, for "said" read --smokeless powder--; and that the said Letters Patent should be read with this correction therein that the same may conform to the record of the case in the Patent Office.

Signed and sealed this 16th day of May, A. D. 1944.

(Seal)

Leslie Frazer  
Acting Commissioner of Patents.

CERTIFICATE OF CORRECTION.

Patent No. 2,342,204.

February 22, 1944.

BILL HARRY MACKEY.

It is hereby certified that error appears in the printed specification of the above numbered patent requiring correction as follows: Page 3, first column, line 1, for "macrated" read --macerated--; and second column, line 23, claim 2, for "said" read --smokeless powder--; and that the said Letters Patent should be read with this correction therein that the same may conform to the record of the case in the Patent Office.

Signed and sealed this 16th day of May, A. D. 1944.

Leslie Frazer  
(Seal) Acting Commissioner of Patents.